

Patented Feb. 9, 1926.

1,572,354

# UNITED STATES PATENT OFFICE.

JAMES H. GRAVELL, OF ELKINS PARK, PENNSYLVANIA.

## RUSTPROOFING BATH FOR IRON AND STEEL.

No Drawing. Application filed May 9, 1922, Serial No. 559,599. Renewed November 3, 1925.

To all whom it may concern:

Be it known that I, JAMES H. GRAVELL, a citizen of the United States, residing at Elkins Park, in the county of Montgomery 5 and State of Pennsylvania, have invented a new and useful Improvement in Rust-proofing Baths for Iron and Steel, of which the following is a specification.

This invention relates to rust proofing 10 iron and steel and the object of the invention is to provide an improved bath compound for the purpose, whereby the rust proofing may be done more effectively and less care need be exercised in maintaining the bath in 15 proper working condition.

According to the rust proofing process to which this invention is applicable, the articles to be rust proofed are immersed in a hot, weak solution of phosphoric acid and water until a substantial coating of iron phosphate is formed and the time required varies, in practice, from one to several hours.

This process is satisfactory where the surface of the articles is perfectly free from acids, for example, where the metal articles have been sand blasted, but where the work has been prepared for rust proofing by pickling there is sufficient acid carried over 20 with the work to contaminate the rust proofing bath. I have discovered that these evil effects of pickling baths, perspiration and the like can be overcome by dissolving 25 metallic sodium in the phosphoric acid prior to mixing it with the water or by dissolving it in the rust proofing bath after the latter 30 has been made up.

To prepare phosphoric acid for a rust 35 proofing bath I use:

|                       | Pounds. |
|-----------------------|---------|
| Phosphoric acid (85%) | 100     |
| Metallic sodium       | 4       |

40 The sodium dissolves forming monosodium phosphate in the acid.

The prepared acid thus formed is used

in the regular way in preparing the rust proofing bath.

The sodium in the solution changes the 50 free sulphuric and other pickling and like acids into the sodium salts of these acids and these salts remain dissolved in the solution and do not precipitate to form a sludge at the bottom of the tanks. The ill effects 55 of the foreign acids are destroyed without danger of causing a sludge to form on the work or to accumulate in the bottom of the tank.

My compound is used in the same way as 60 unprepared phosphoric acid and meets all the requirements even when manganese dioxide or zinc phosphate or both are added to the bath which is often done in practice.

It will be evident to those skilled in the 65 art that the metallic sodium may be replaced by chemical equivalents such as mono-, di-, or tri-sodium phosphate without departing from the spirit of the invention, and the phosphoric acid may be made from 70 material containing sodium so proportioned that the requisite amount of sodium will be present in the phosphoric acid when it is manufactured. My experience indicates that magnesium and potassium may be used 75 instead of the sodium and it is understood that in the claims the term "sodium" includes also magnesium and potassium, or combinations of sodium, magnesium and potassium.

80 I claim:

1. A bath for rust proofing comprising water, free phosphoric acid and mono-sodium phosphate which combining with pickling and foreign acids opposes the formation of a sludge.

2. The method of rust proofing a metallic surface which consists in forming a substantial coating of iron phosphate on the surface by subjecting the surface to the 85 action of a bath containing mono-sodium phosphate, free phosphoric acid and water, substantially as described.

JAMES H. GRAVELL